

# United States Patent

Sakamoto et al.

[15] 3,637,393

[45] Jan. 25, 1972

[54] **LIGHT-SENSITIVE COLOR  
PHOTOGRAPHIC MATERIAL WITH  
REDUCED FOG AND NO DECREASE IN  
SPEED DURING DEVELOPMENT**

[72] Inventors: Kenro Sakamoto; Isamu Fushiki; Shinichi Nakamura, all of Tokyo, Japan

[73] Assignee: Konishiroku Photo Industry Co., Ltd., Tokyo, Japan

[22] Filed: July 9, 1970

[21] Appl. No.: 53,657

[30] **Foreign Application Priority Data**

July 10, 1969 Japan.....44/54116

[52] U.S. Cl.....96/109, 96/100, 96/120,

96/122, 96/125

[51] Int. Cl.....G03c 1/34

[58] Field of Search.....96/109, 120, 125, 100, 122

[56]

**References Cited**

**UNITED STATES PATENTS**

|           |         |                   |        |
|-----------|---------|-------------------|--------|
| 2,465,149 | 3/1949  | Dersch et al..... | 96/109 |
| 2,728,659 | 12/1955 | Lorin et al.....  | 96/109 |
| 2,981,624 | 4/1961  | Dersch et al..... | 96/109 |

Primary Examiner—Norman G. Torchin  
Assistant Examiner—Alfonso T. Suro Pico  
Attorney—Waters, Roditi, Schwartz & Nissen

[57]

**ABSTRACT**

Fog is reduced and speed is maintained during development of light-sensitive color photographic materials which comprise at least one of certain mercaptotetrazole compounds and at least one of several hydroquinone compounds.

7 Claims, No Drawings





## Examples of the Compound (II):



30 Both the compounds (I) and compounds (II) of the present invention may be used in admixture of two or more so as to be in conform to the purpose of application of the resulting photographic materials. The compounds (I) and (II) may be 35 incorporated into one layer or may separately be incorporated into adjacent layers. These compounds may be incorporated not only into emulsion layers but also into auxiliary layers such as sub layer, inter layer, protective layer and the like. Further, the compounds may be added to a silver halide emulsion at 40 any stage during the preparation thereof, but it is more effective to add the compounds at a stage during the second ripening or a stage prior to coating the emulsion to a support.

The amounts of the compounds to be added are not particularly limited, and the optimum amounts thereof vary depending 45 on the kinds of the compounds. Generally, however, the amounts of the compounds (I) and (II) are preferably  $10^{-6}$  to  $10^{-1}$  moles and  $10^{-6}$  to  $10^{-1}$  moles, respectively, per mole of silver halide. Among the compounds (I) and (II), those which are lipophilic are added in the form of solutions in a high boiling 50 organic solvent such as dibutyl phthalate or the like or in a low boiling organic solvent such as chloroform, acetone, dimethylformamide or the like, while those which are water-soluble are added in the form of solutions in a water-miscible organic solvent or an aqueous alkali solution.

55 The photographic emulsion used in the present invention include AgCl, AgBr, AgClBr, AgBrI and the like. The emulsion may be optically sensitization treatment with a cyanine or merocyanine dye or to chemically sensitized treatment with a sulfur-containing compound (sodium thiosulfate), noble 60 metal salt (gold chloride), polyalkylene oxide derivative, reducing compound or the like. Further, the emulsion may have been incorporated with such a hardener as formalin and such a coating aid as a synthetic or natural surface active agent, e.g., saponin. The color couplers which are used in the 65 present invention are those which develop colors through the reaction with a p-phenylenediamine color developer. Generally, there may be used a yellow coupler having a benzoylacetanilide group, a magenta coupler having a pyrazolone or indazolone group, and a cyan coupler having a 70 phenol or naphthol group. These couplers may contain in the active methylene- or methine-portion a substituent capable of releasing by color development reaction, e.g., a halogen or an arylazo, aryloxy or the like group. Further, the couplers may contain in the molecule either one or both of a ballasting 75 group, e.g., a long chain alkyl group or an alkylphenoxy group,



TABLE 2

| Compound (I)    | Compound (II)   | Relative speed | Fog  |
|-----------------|-----------------|----------------|------|
| Compound (I)-2  | Compound (II)-2 | 100            | 0.12 |
|                 | Compound (II)-4 | 116            | 0.11 |
|                 | Compound (II)-9 | 115            | 0.09 |
| Compound (I)-7  | Compound (II)-2 | 131            | 0.09 |
|                 | Compound (II)-4 | 100            | 0.10 |
|                 | Compound (II)-9 | 122            | 0.10 |
| Compound (I)-13 | Compound (II)-2 | 124            | 0.09 |
|                 | Compound (II)-4 | 138            | 0.07 |
|                 | Compound (II)-9 | 100            | 0.12 |
| Compound (I)-18 | Compound (II)-2 | 113            | 0.12 |
|                 | Compound (II)-4 | 119            | 0.10 |
|                 | Compound (II)-9 | 128            | 0.09 |
| Compound (I)-18 | Compound (II)-2 | 108            | 0.12 |
|                 | Compound (II)-4 | 118            | 0.11 |
|                 | Compound (II)-9 | 119            | 0.11 |

From the results shown in table 2, it is understood that every combination gives a light-sensitive photographic material higher in speed and less in fog than in the case where the compound (I) is used alone.

## EXAMPLE 3

The same high speed silver bromoiodide photographic emulsion as in example 1 was incorporated with  $3.1 \times 10^{-4}$  moles/mole AgX of a sensitizing dye having the structure shown below to obtain a green light-sensitive emulsion.



Subsequently,  $9 \times 10^{-4}$  moles/mole AgX of the compound (II)-9 was added to the emulsion. Thereafter, a magenta coupler of the structure shown below was dispersed in the thus treated emulsion by means of a high speed rotary mixer to form a dispersion.



The dispersion had the composition shown below in which the amounts of the constituents were per mole of AgX.

| Composition of dispersion |         |
|---------------------------|---------|
| Coupler                   | 56 g.   |
| Tricresyl phosphate       | 25 g.   |
| Ethyl acetate             | 30 g.   |
| 2% Gelatine               | 500 ml. |
| 5% Alkanol B              | 21 cc.  |

Subsequently, the dispersion was coated on a cellulose triacetate film to a dry thickness of  $5\mu$  and then dried to form an emulsion layer on the film. Onto this emulsion layer, each of dispersions of protective layers 1 and 2 of the compositions shown below was coated to a dry thickness of  $1\mu$ , and then dried.

Compositions of protective layers

|                   | Protective layer 1 | Protective layer 2 |
|-------------------|--------------------|--------------------|
| Compound (II)-7   | 0                  | 5.0 g.             |
| Dibutyl phthalate | 2.0 g.             | 2.0 g.             |
| Ethyl acetate     | 5.0 g.             | 5.0 g.             |
| 2% Gelatine       | 800 ml.            | 800 ml.            |
| 5% Alkanol B      | 7.5 ml.            | 7.5 ml.            |

The film after drying was subjected to the same color development treatment as in example 1 and measured in density by means of a green filter to obtain the results set forth in table 3.

TABLE 3

|                                                     | Relative speed | Fog  |
|-----------------------------------------------------|----------------|------|
| Protective layer 1 (control)                        | 100            | 0.11 |
| Protective layer 2 [containing the compound (II)-7] | 126            | 0.10 |

This example shows the case where the compound (I) was added to the emulsion layer and the compound (II) was added to the protective layer. However, the same effects as above can be obtained also in the case where, conversely, the compound (II) is added to the emulsion layer and the compound (I) is added to the protective layer.

## EXAMPLE 4

A high-speed silver bromoiodide photographic emulsion (containing 4.5 mole % of AgI and 180 g./mole AgX of gelatine) was subjected to second ripening. To this emulsion were added  $2 \times 10^{-4}$  moles/mole AgX of 5-methyl-7-hydroxy-1,3,4-triaza-1,2-dihydro-5H-1,3,4-triaza-7-oxoindolizine and  $1.3 \times 10^{-3}$  moles/mole AgX of the compound (I)-5. Subsequently, a yellow coupler of the structure shown below was dissolved in caustic soda and water and added in an amount of  $1.3 \times 10^{-1}$  moles/mole AgX.



Thereafter, each of dispersions 1 and 2 of the compositions shown below was mixed with the above-mentioned emulsion, and the resulting mixture was coated on a film base to dry thickness of  $4.0\mu$  and then dried. In the dispersions, the amounts of the constituents were per mole of AgX.

Compositions of dispersions

|                 | Dispersion 1 | Dispersion 2 |
|-----------------|--------------|--------------|
| Compound (II)-8 | 0            | 4 g.         |
| Ethyl acetate   | 8 g.         | 8 g.         |
| 2% Gelatine     | 600 ml.      | 600 ml.      |
| 5% Alkanol B    | 18 ml.       | 18 ml.       |

The film after drying was subjected to definite exposure through an optical wedge and then to development at  $20^\circ\text{C}$ . for 10 minutes with the color developer shown below to obtain the results set forth in table 4. The bleaching and fixing treatments were effected in the same manner as in example 1.

Color developer

|                                           |           |
|-------------------------------------------|-----------|
| Anhydrous sodium sulfite                  | 2.0 g.    |
| 4-amino-N,N'-diethylaniline hydrochloride | 5.0 g.    |
| Sodium carbonate (monohydrate)            | 50.0 g.   |
| Potassium bromide                         | 1.0 g.    |
| Water to make                             | 1,000 ml. |

TABLE 4

|                                               | Relative speed | Fog  |
|-----------------------------------------------|----------------|------|
| Dispersion 1 (control)                        | 100            | 0.15 |
| Dispersion 2 [containing the compound (II)-8] | 119            | 0.11 |

Thus, in all the cases where the present invention is practiced in the above manner, the amount of fog formed is less than in the cases where the combinations of the said two compounds were not used, and obvious sensitizing effects are observed.

What we claim is:

1. A light-sensitive gelatinous silver halide color photographic material characterized by containing in at least one of the layers constituting the photographic material at least one mercaptotetrazole compound of the general formula,



wherein  $\text{R}_1$ ,  $\text{R}_2$  and  $\text{R}_3$  are individually a hydrogen atom, an alkyl, aryl or aralkyl group, provided that  $\text{R}_2$  and  $\text{R}_3$  may be same or different, and at least one hydroquinone compound of the general formula,



wherein  $\text{R}_4$  is an alkyl group having 1 to 18 carbon atoms, and  $\text{R}_5$ , which is in the 5- or 6-position, is a hydrogen atom or an alkyl group having 1 to 18 carbon atoms.

2. A light-sensitive gelatinous silver halide color photographic material as claimed in claim 1, wherein said mercaptotetrazole compound and said hydroquinone compound jointly exist in a same layer selected from the emulsion layer, inter layer, sub layer, filter layer and protective layer of the photographic material.

3. A light-sensitive gelatinous silver halide color photographic material as claimed in claim 1, wherein said mercap-

20

25

30

35

45

50

55

60

65

70

75

totetrazole compound and said hydroquinone compound separately exist in the adjacent layers selected from the emulsion layer, inter layer, sub layer, filter layer and protective layer of the photographic material.

4. A light-sensitive gelatinous silver halide photographic material as claimed in claim 1, wherein either one or both of said mercaptotetrazole compound and said hydroquinone compound are used in combination with a chemical sensitizer or/and an optical sensitizer.

5. A light-sensitive gelatinous silver halide color photographic material as claimed in claim 1, wherein a color coupler is also incorporated in the emulsion layer of said photographic material.

6. A light-sensitive gelatinous silver halide color photographic material as claimed in claim 1, wherein said mercaptotetrazole compound is



and said hydroquinone compound is



7. A light-sensitive gelatinous silver halide color photographic material as claimed in claim 1, wherein said mercaptotetrazole compound is



40 and said hydroquinone compound is



\* \* \* \* \*